

1

3,532,499

AMINO - N - OXIDES AS DEVELOPMENT  
ACCELERATORS IN PHOTOGRAPHY  
Jozef Frans Willems, Wilrijk-Antwerp, Francis Jeanne  
Sels, Kontich, and Joseph Louis DeMunck, Heide-  
Kalmthout, Belgium, assignors to Gevaert-Agfa N.V.,  
Mortsel, Belgium, a company of Belgium  
No Drawing. Filed Aug. 22, 1966, Ser. No. 573,801  
Claims priority, application Great Britain, Oct. 7, 1965,  
42,592/65

Int. Cl. G03c 5/30, 1/06, 1/48  
U.S. Cl. 96—66.3

7 Claims

## ABSTRACT OF THE DISCLOSURE

Photographic light-sensitive silver halide emulsions containing an onium derivative of an amino-N-oxide are described. The onium derivatives of amino-N-oxides are development accelerators, extend the development latitude within normal developing times in which screen prints of good quality can be produced and do not fog.

This invention relates to the development of photographic silver halide emulsions in the presence of substances influencing the development and combinations of these substances with known development accelerators.

It is known that the development of continuous tone images by means of a hydroquinone p-N-methyl-aminophenol developer is accelerated under the influence of polyoxyalkylene compounds having a molecular weight preferably above 1500. When, however, such polyoxyalkylene compounds are used in combination with a hydroquinone-formaldehyde-bisulphite developer, as is known from the German Pat. No. 1,141,531 filed Jan. 24, 1962 by Perutz Photowerke G.m.b.H., an increase of the gradation together with a desensitisation is obtained. The latter combination is found to be very suitable for the development of light-sensitive materials suited for use in the graphic art on account of the very contrasty development obtained therewith.

It is also known that the development retardation caused when using the combination of polyoxyalkylene compounds with the above-mentioned type of developer can be counteracted and that the initial rate of development can be raised by using quaternary ammonium salts in conjunction with the above combination. It is, however, also known that quaternary ammonium compounds, when used in photographic emulsion layers tend to increase the fog considerably.

An enhanced initial rate of development and a development interval as long as possible in which sharp screen dots can be obtained yet, are of importance in practice for the development of graphic reproductions.

It has been found now that onium derivatives of amino-N-oxides and more particularly compounds according to the following structural formulae:



2



wherein:

each of  $R_1$  and  $R_2$  represents an alkyl radical e.g. methyl, an aralkyl radical e.g. benzyl, or together represent the atoms required for completing an heterocyclic ring e.g. a morpholine, a pyrrolidine, or a piperidine ring,

$R_3$  represents an alkyl radical e.g. ethyl or an aralkyl radical e.g. benzyl,

$R_4$  represents alkyl and aralkyl,

$R_5$  represents a hydrogen atom or a substituent such as an alkyl radical or an aralkyl radical,

$X^-$  represents an anion,

$R$  represents a bivalent organic radical such as an alkylene radical or an alkylenephenylenealkylene radical, and

$Z$  represents the atoms required for forming an heterocyclic ring system,

are not only very efficient development accelerators by themselves, but they also considerably increase the initial rate of development of a developer combination comprising hydroquinone and polyoxyalkylene compounds and extend the development latitude within normal developing times, in which screen prints of good quality can be produced.

Compounds corresponding to one of these general formulae are i.e. the compounds resulting from the alkylation of tertiary amino-N-oxides such as trimethylamino-N-oxide, triethylamino-N-oxide, tributylamino-N-oxide, monomethyldiethylamino - N - oxide, dodecyldimethylamino-N-oxide, cetyltrimethylaminio-N-oxide, pyridine-N-oxide,  $\alpha$ -,  $\beta$ -, or  $\gamma$ -picoline-N-oxide, chloropyridine-N-oxide, quinoline-N-oxides, lepidine-N-oxides, and amino-N-oxides derived from other heterocyclic nitrogen compounds.

Suitable alkylating agents are, e.g., alkyl bromides, alkyl tolsulphonates, alkylmethyl sulphonates, aralkyl bromides, 1,2-dibromomethane, 1,4-dibromobutane, p-xylylene dibromide,  $N,N'$ -bis-(2-bromoethyl)-succinamide, bis-(2-bromoethyl)-sulphone, bis - (2 - bromoethyl)-sulphide, bis - (2 - bromoethyl) - ether, and  $N,N'$ -bis-(10-bromohendecanoyl)-ethylenediamine.

By way of illustration the preparation of some of the compound according to the above general formulae will now be described.

## Preparation 1



In a 250 cm.<sup>3</sup> flask fitted with a condenser 0.25 mole of ethylene dibromide is mixed with 0.5 mole of  $\beta$ -picoline-N-oxide in 150 cm.<sup>3</sup> of ethanol. After refluxing for 5 hours the solvent is evaporated in vacuo. The residue is recrystallised from a mixture of ethanol and tetrahydrofuran (50:50). Melting point: 170° C. (decomposition).

## Preparation 2



In a 250 cm.<sup>3</sup> flask fitted with a condenser 0.25 mole of ethylene dibromide is mixed with 0.5 mole of  $\gamma$ -picoline-N-oxide in 150 cm.<sup>3</sup> of ethanol. After refluxing for 13 hours the solvent is evaporated in vacuo. The residue is recrystallised from a mixture of ethanol and tetrahydrofuran (50:50). Melting point: 170° C. (decomposition).

## Preparation 3



In a 250 cm.<sup>3</sup> flask fitted with a condenser 0.25 mole of ethylene dibromide is mixed with 0.5 mole of  $\alpha$ -picoline-N-oxide in 150 cm.<sup>3</sup> of ethanol. After refluxing for 15 hours the solvent is evaporated in vacuo. The residue is washed with acetone and then recrystallised from its 95% solution of ethanol. Melting point: 230° C. (decomposition).

## Preparation 4



In a 250 cm.<sup>3</sup> flask fitted with a condenser 0.05 mole of xylylene dibromide is admixed with 0.12 mole of triethylamine-N-oxide in 150 cm.<sup>3</sup> of acetone. After having been refluxed for 2 hours the reaction mixture is cooled and the precipitate formed is filtered by suction. This precipitate is washed two times with boiling acetone. Melting point: 230° C. (decomposition).

## Preparation 5



In a 100 cm.<sup>3</sup> flask fitted with a condenser 0.05 mole of tetramethylene dibromide is mixed with 0.12 mole of triethylamine-N-oxide in 15 cm.<sup>3</sup> of acetone. After having been refluxed for 5 hours the precipitate is filtered by suction and washed with chloroform and afterwards with ether. Melting point: explodes on the Kofler hot bench at 200° C.

## Preparation 6



In a 100 cm.<sup>3</sup> flask fitted with a condenser 0.1 mole of dodecylmethyl sulphonate is mixed with 0.1 mole of pyridine-N-oxide in 65 cm.<sup>3</sup> of acetonitrile. After refluxing the solution for 6 hours, the solvent is evaporated in vacuo and the waxy residue is washed with ether.

## Preparation 7



In a 100 cm.<sup>3</sup> flask fitted with a condenser 0.05 mole of hexadecylmethyl sulphonate is mixed with 0.05 mole of pyridine-N-oxide in 70 cm.<sup>3</sup> of acetonitrile. After refluxing the solution for 6 hours, the solvent is evaporated in vacuo and the waxy residue is washed with ether.

## Preparation 8



In a 100 cm.<sup>3</sup> flask fitted with a condenser 0.1 mole of hexamethylene dibromide is mixed with 0.2 mole of pyridine-N-oxide in 40 cm.<sup>3</sup> of acetonitrile. After having been refluxed for 2 hours the formed precipitate is filtered by suction. The precipitate is recrystallised from ethanol. Melting point: 162° C.

## Preparation 9



In a 100 cm.<sup>3</sup> flask fitted with a condenser 0.1 mole of n-hexylmethyl sulphonate is mixed with 0.1 mole of pyridine-N-oxide in 50 cm.<sup>3</sup> of acetonitrile. After refluxing the solution for 6 hours, the solvent is evaporated in vacuo and the waxy residue is washed with a mixture of ether and ethyl acetate (50:50).

## Preparation 10



In a 100 cm.<sup>3</sup> flask fitted with a condenser 0.1 mole of n-octylmethyl sulphonate is mixed with 0.1 mole of pyridine-N-oxide in 50 cm.<sup>3</sup> of acetonitrile. After refluxing the solution for 6 hours, the solvent is evaporated in vacuo and the waxy residue is washed with ether.

## Preparation 11



In a 100 cm.<sup>3</sup> flask fitted with a condenser 0.1 mole of n-decylmethyl sulphonate is mixed with 0.1 mole of pyridine-N-oxide in 50 cm.<sup>3</sup> of acetonitrile. After refluxing the solution for 6 hours, the solvent is evaporated and the waxy residue is washed with ether.

The product according to the formula:



is prepared as described in J. Org. Chem. 22 (1957) p. 1135. The product according to the formula:



is prepared as described in J. Chem. Soc. (1956) p. 2407.

The following products are prepared as described in Acta Chem. Scand. 17 (1963) p. 953:





The onium derivatives of the amino-N-oxides influencing the rate of development are preferably added to the light-sensitive silver halide emulsions in dissolved form in water or a mixture of water and water-miscible organic solvents, which do not impair the photographic characteristics of the emulsion.

However, these condensation products can also be incorporated into the emulsion by imbibition by treating it with a solution containing these products or by diffusion from an adjacent water-permeable layer comprising these products.

The onium derivatives of the amino-N-oxides used according to the present invention can be added to the light-sensitive silver halide emulsion during different preparation steps of the light-sensitive material. For example they can be incorporated therein by a separate addition or they can be added as a mixture with one or more ingredients used in the formation of the silver halide grains, during the physical or chemical ripening or during another step preceding the coating of the emulsion. For the purpose of increasing the gradation and accelerating the development the said derivatives are preferably used in combination with water-soluble alkylene oxide condensation products as described e.g. in the United States patent specifications 1,970,578 by Conrad Schoeller and Max Wittwer issued Aug. 21, 1934, 2,240,472 by Donald R. Swan issued Apr. 29, 1941, 2,423,549 by Ralph K. Blake, William A. Stanton, Ferdinand Schulze issued July 8, 1947, 2,441,389 by Ralph K. Blake issued Mar. 11, 1948, 2,531,832 by William A. Stanton issued Nov. 11 1950, 2,533,990 by Ralph K. Blake issued Dec. 12, 1950 and the British patent specifications 920,637 filed May 7, 1959 by Gevaert Photo-Producten N.V., 940,051 filed Nov. 1, 1961 by Gevaert Photo-Producten N.V., 945,340 filed Oct. 23, 1961 by Gevaert Photo-Producten N.V., 991,608 filed June 14, 1961 by Kodak and the Belgian patent specification 648,710 filed June 2, 1964 by Gevaert Photo-Producten N.V.

The polyoxyalkylene compounds i.e. alkylene oxide condensation products together with the onium derivatives of the amino-N-oxides as described above can be added to the composition of the silver halide emulsion of to a water-permeable layer, which together with the emulsion layer forms part of a water-permeable element.

The said derivatives are preferably added to the emulsion after the chemical ripening and just before the coating of the emulsion.

The alkylene oxide condensation products and/or the onium derivatives of the amine-N-oxides can also be added to the developing bath.

The optimum amount of alkylene oxide condensation product and onium derivatives of amine-N-oxides according to the above formulae depends on the very compound, on the nature of the colloid binder of the silver halide grains and on the amount and type of silver halide in the emulsion. In general, however, the above alkylene oxide condensation products are added to the light-sensitive material in an amount of 100 mg. of 10 g. per mole of silver halide. When incorporated into the developer they are used in amounts ranging from 100 mg. to 10 g. per litre of developer. The amount of onium derivative incorporated into the light-sensitive material preferably ranges between 5 mg. and 5 g. per mole of silver halide. When added to the developing bath the derivative is used preferably in an amount varying between 5 mg. to 5 g. per litre.

The development acceleration and the increase of dot definition and of the development latitude obtained with the products according to the present invention can be combined with a chemical sensitisation by using in combination with the above-mentioned onium derivatives of amine-N-oxides chemical sensitising agents such as sulphur-containing compounds e.g. allyl isothiocyanate, allyl thiourea, or sodium thiosulphate, reducing agents such as the tin compounds described in the Belgian patent specification 493,464 filed Jan. 24, 1950 and 568,687 filed June 18, 1958 by Gevaert Photo-Production, N.V., the iminoaminomethane sulphonic acid compounds described in the British patent specification 789,823 filed Apr. 29, 1955 by Gevaert Photo-Producten N.V., or precious metal compounds such as gold, platinum, palladium, iridium, ruthenium, and rodium compounds. The sensitising action also manifests itself of course, when combining the above-mentioned condensation products with the sensitising compounds present by nature in gelatin.

The products influencing the development according to the present invention can also be used in combination with stabilising agents for silver halide emulsions, such as mercury compounds and the compounds described in the Belgian patent specifications 571,916 and 571,917 both filed Oct. 10, 1958 by Gevaert Photo-Producten N.V., and in combination with sensitising and stabilising cadmium salts in the light-sensitive material as well as in the developer.

The onium compounds of amine-N-oxides either or not in combination with polyoxyalkylene compounds may be used to improve the developing characteristics of various types of emulsions. So, they may be used in combination with optically sensitised emulsion as well as with not optically sensitised emulsions e.g. X-ray emulsions as well as orthochromatic and panchromatic emulsions, and emulsions sensitive to infrared radiation. Various silver salts may be used as light-sensitive salt e.g. silver bromide, silver iodide, silver chloride, or mixed silver halides such as silver chlorobromide or silver bromoiodide. Said compounds may be used in emulsions for colour photography, emulsions of the mixed packet type, or emulsions of the mixed grain type. They can also be used in emulsions, which form latent images predominantly on the surface of the silver halide crystal, or in emulsions, which form latent images predominantly inside the silver halide crystal. They may be used in silver halide emulsions for application in the silver halide diffusion transfer process or other transfer processes based on silver halide photography, in which e.g. the diffusion of a developer, a coupler, or a dye is applied.

Together with the above-mentioned products, derivatives of tetra-azaindenes having the following general for-

formula can be used as fog-inhibiting compounds in the light-sensitive material:



wherein:

each of R'1 and R'2 represents a hydrogen atom, an alkyl, an aralkyl, or an aryl radical, and R'3 represents a hydrogen atom, an alkyl, a carboxy, or an alkoxy carbonyl group.

Such compounds can be prepared by starting from 1 mole of  $\beta$ -ketoester of an  $\alpha$ -ethoxymethylene- $\beta$ -ketoester with 1 mole of a suitable 3-amino-1,2,4-triazole. By way of example of such derivative 5-methyl-7-hydroxy-s-triazolo(1,5-a)-pyrimidine can be mentioned.

Other agents such as hardening agents, wetting agents, plasticisers, developing agents, optical sensitising agents, and binders such as gelatin, latices, etc. can be incorporated into the emulsion in the usual way.

The combination of the alkylene oxide derivatives influencing the development and onium derivatives of amine-N-oxides according to the present invention can preferably be used in the development of silver chloride and silver bromochloride emulsions with a hydroquinone-formaldehyde-bisulphite developer.

The following examples illustrate the invention.

#### EXAMPLE 1

A washed gelatin silver iodobromide emulsion (94.5 mole percent of silver bromide and 5.5 mole percent of

Boric acid—5 g.  
Potassium bromide—0.5 g.  
Water to—1 litre.

The sensitometric results stated in Table 1 present a clear picture of the development acceleration.

TABLE 1

|    | Onium compound of preparation No. | Added amount in mg. per kg. of emulsion ready for coating | Speed log i.t. of above fog value | Gamma | Fog  |
|----|-----------------------------------|-----------------------------------------------------------|-----------------------------------|-------|------|
| 10 |                                   |                                                           | 1.31                              | 0.47  | 0.08 |
| 10 |                                   | 303                                                       | 1.18                              | 0.47  | 0.08 |
| 11 |                                   | 331                                                       | 1.15                              | 0.50  | 0.09 |
| 15 | 6                                 | 359                                                       | 1.15                              | 0.50  | 0.09 |

#### EXAMPLE 2

Test strips with a light-sensitive silver halide emulsion of the positive type (average grain size:  $0.35\mu$ ; comprising 98 mols percent of silver bromide and 2 mole percent of silver iodide) are exposed in identical conditions and developed for different times in a solution having the following composition:

|                             | G.  |
|-----------------------------|-----|
| 25 Sodium hexametaphosphate | 1   |
| Anhydrous sodium sulphite   | 20  |
| Anhydrous sodium carbonate  | 20  |
| Potassium bromide           | 0.5 |
| 30 Hydroquinone             | 4.4 |

The development accelerators listed in Table 2 are added to samples of this solution. The table also denotes the densities obtained after different development times.

TABLE 2

| Onium compound according to the formula | Added amount in mg. per litre | Density obtained after developing for |         |         |         |
|-----------------------------------------|-------------------------------|---------------------------------------|---------|---------|---------|
|                                         |                               | 15 sec.                               | 30 sec. | 45 sec. | 60 sec. |
|                                         | 0.00                          | 0.00                                  | 0.65    | 0.10    |         |
|                                         | 135                           | 0.15                                  | 0.55    | 1.10    | 1.60    |
|                                         | 140                           | 0.45                                  | 1.20    | 1.75    | 2.10    |

silver iodide), (average grain size of the silver halide:  $0.8\mu$ ) of the negative type is ripened at  $45^\circ C$ .

The emulsion ready for coating contains per kg. 50 g. of silver halide, 75 g. of gelatin, 30 mg. of optical sensitising agent according to the following structural formula:



50 mg. of 5-methyl-7-hydroxy-s-triazolo(1.5-a)-pyrimidine as a stabilising agent, and 500 mg. of saponine as a wetting agent. The emulsion is applied to a cellulose triacetate support and dried. Other test strips are prepared by adding to samples of the above-mentioned emulsions prior to the coating step the development accelerators in the amounts listed in the table hereinafter.

All of the test strips are exposed in identical conditions through a grey wedge and developed for 7 minutes in the following solution:

Water—800 cm.<sup>3</sup>  
Monomethyl-u-aminophenol sulphate—2 g.  
Hydroquinone—5 g.  
Anhydrous sodium sulphite—100 g.  
Borax—10 g.

50 The amounts of compounds influencing the development, defined in Table 3, are added before the coating step to samples of a green-sensitised gelatin silver chlorobromide emulsion (35 mole percent of bromide) comprising 5-methyl-7-hydroxy-s-triazolo-(1,5-a)-pyrimidine, cadmium chloride and 25% by weight of a latex plasticizer calculated on the weight of gelatin. The latex-plasticizer consists of a latex of a 20% by weight aqueous dispersion of poly(ethyl acrylate) prepared according to known techniques of emulsion polymerisation by carrying out the polymerisation in the presence of 8% by weight (calculated on the monomer) of an emulsifying agent of one of the following types: the condensation product of oleic acid and methyltaurine, the sodium salt of laurylsulphonic acid, or the sodium salt of an alkylbenzene sulphonic acid wherein the alkyl radical contains from 8 to 12 carbon atoms.

55 Subsequently the emulsion strips are hardened with formaldehyde each time applied in the same way to a cellulose triacetate support, and dried. They are exposed then through a continuous wedge and a glass screen to light with a colour temperature of  $3700^\circ K$ . The exposure is regulated so that the wedge print of the screen includes the beginning of dot formation as well as the disappearance of the high lights.

60 The dot sharpness is judged of visually by comparison to standard materials, which is decreasing value of dot

sharpness quality are defined with the numbers 1, 2, 3, and 4.

Development is carried out at 19° C. in a developing bath comprising:

|                                  | G.  | 5  |
|----------------------------------|-----|----|
| Sodium bisulphite                | 1.5 |    |
| Hydroquinone                     | 17  |    |
| Formaldehyde bisulphite          | 60  |    |
| Anhydrous sodium carbonate       | 60  |    |
| Anhydrous sodium bicarbonate     | 15  | 10 |
| Potassium bromide                | 1   |    |
| Water to 1000 cm. <sup>3</sup> . |     |    |

X represents an anion, R represents a bivalent organic radical such as an alkylene or an alkylene-phenylene-alkylene, and Z represents the atoms required for forming a pyridine or quinoline nucleus.

2. A photographic light-sensitive silver halide material containing an onium derivative of an amino-N-oxide corresponding to one of the following structural formulae:



TABLE 3

| Compound                                                   | Mg. per mol of silver halide | Development time (in min.) |    |       |     |     |       | Dot definition |                            |      |
|------------------------------------------------------------|------------------------------|----------------------------|----|-------|-----|-----|-------|----------------|----------------------------|------|
|                                                            |                              | 1.5                        |    | 2.5   |     | 3.5 |       | 1.5            | 2.5                        | 3.5  |
| γ                                                          | Speed                        | Fog                        | γ  | Speed | Fog | γ   | Speed | Fog            | Development time (in min.) |      |
| Polyethylene glycol having an average mol. weight of 2,000 | 120                          | 3.9                        | 24 | 0.01  | 6.7 | 87  | 0.01  | 5.7            | 100                        | 0.01 |
| A mixture of compound A <sup>1</sup> and                   | 120                          | >10                        | 12 | 0.01  | >10 | 47  | 0.01  | >10            | 62                         | 0.01 |
| A mixture of compound B <sup>2</sup> and                   | >10                          |                            | 35 | 0.01  | >10 | 60  | 0.01  | >10            | 76                         | 0.01 |
| A mixture of compound A and                                | 120                          | >10                        | 32 | 0.01  | >10 | 65  | 0.01  | >10            | 80                         | 0.10 |
| The compound prepared according to preparation 4           | 200                          | >10                        | 32 | 0.01  | >10 | 65  | 0.01  | >10            | 80                         | 0.10 |
| A mixture of compound A and                                | 120                          | 10.5                       | 25 | 0.01  | 9.4 | 81  | 0.01  | 8.4            | 107                        | 0.01 |
| The compound prepared according to preparation 4           | 200                          |                            |    |       |     |     |       |                | 3                          | 1    |
|                                                            |                              |                            |    |       |     |     |       |                |                            | 2    |

NOTE.—The relative speed is expressed on a percentage basis, the exposure value having been measured at a density 3 above fog value.



prepared from 2 mole of methoxypolyethylene glycol and 1 mole of OCN—(CH<sub>2</sub>)<sub>6</sub>—NCO.



We claim:

1. Process for developing photographic materials containing a light-sensitive silver halide wherein the development is carried out in the presence of an onium derivative of an amino-N-oxide corresponding to one of the following structural formulae:



wherein

each of R<sub>1</sub> and R<sub>2</sub> represents an alkyl radical, an aralkyl radical, or together the atoms required for completing an heterocyclic ring,

R<sub>3</sub> represents an alkyl radical or an aralkyl radical,

R<sub>4</sub> represents an alkyl radical or an aralkyl radical,

R<sub>5</sub> represents a hydrogen atom, an alkyl radical or an aralkyl radical,

70

75 wherein:

wherein:

each of R<sub>1</sub> and R<sub>2</sub> represents an alkyl radical, an aralkyl radical, or together the atoms required for completing an heterocyclic ring,

R<sub>3</sub> represents an alkyl radical or an aralkyl radical, R<sub>4</sub> represents an alkyl radical or an aralkyl radical, R<sub>5</sub> represents a hydrogen atom, an alkyl radical or an aralkyl radical,

X<sup>-</sup> represents an anion,

R represents a bivalent organic radical such as an alkylene or an alkylene-phenylene-alkylene, and Z represents the atoms required for forming a pyridine or quinoline nucleus.

3. A photographic light-sensitive silver halide material according to claim 2, containing in addition to an onium derivative of an amino-N-oxide a polyoxyalkylene compound.

4. A photographic light-sensitive silver halide material according to claim 3, containing in addition to an onium derivative of an amino-N-oxide a polyoxyalkylene compound and a fog-inhibiting compound of the following general formula:



**11**

each of R'<sub>1</sub> and R'<sub>2</sub> represents a hydrogen atom, an alkyl, aralykl or aryl radical, and R'<sub>3</sub> represents a hydrogen atom, an alkyl, a carboxy, or an alkoxy carbonyl group.

5. Process according to claim 1, wherein an onium derivative is present in the light-sensitive material in a range of 5 mg. to 5 g. per mole of silver halide.

6. The silver halide material according to claim 3, wherein the polyoxyalkylene compound is present in the light-sensitive material in an amount ranging from 100 mg. to 10 g. per mole of silver halide.

7. Process according to claim 1, wherein an onium

derivative is present in a developing bath in an amount varying from 5 mg. to 5 g. per litre.

**References Cited****UNITED STATES PATENTS**

3,129,100 4/1964 Grabhöfer et al. ----- 96—95

NORMAN G. TORCHIN, Primary Examiner

M. FOKELLEY, Assistant Examiner

U.S. Cl. X.R.

96—95

UNITED STATES PATENT OFFICE  
CERTIFICATE OF CORRECTION

Patent No. 3,532,499 Dated October 6, 1970

Inventor(s) Jozef Frans Willems, Francis Jeanne Sels and Joseph Louis DeMunck

It is certified that error appears in the above-identified patent and that said Letters Patent are hereby corrected as shown below:

Column 2, line 52, "cetyltrimethylaminio" should read -- cetyltrimethylamino --. Column 3, line 2, "compound" should read -- compounds --. Column 5, third formula set forth as



line 60, "Mar." should read -- May --. Column 6, line 55, "emulsion" should read -- emulsions --. Column 7, line 72, "Monomethyl-u-amino-phenol" should read -- Monomethyl-p-aminophenol --. Column 8, line 31, "accelerators" should read -- accelerators --; Table 2, under the heading "45 sec.", "0.65" should read -- 0.05 --. Column 9, Table 3, column 2, line 4, insert -- 200 --; Table 3, column 1, last line after "preparation" insert -- 8 --; line 30, the formula set forth as



should read



Column 10, line 1, "X<sub>-</sub>" should read -- X<sup>-</sup> --; claim 2, formula 5 set forth as



claim 3, line 2, "containning" should read -- containing --.

Signed and sealed this 7th day of March 1972.

(SEAL)  
Attest:

EDWARD M.FLETCHER,JR.  
Attesting Officer

ROBERT GOTTSCHALK  
Commissioner of Patents